



US005991591A

**United States Patent** [19]

Chen et al.

[11] **Patent Number:** **5,991,591**[45] **Date of Patent:** **Nov. 23, 1999**[54] **FUSER USING CERAMIC ROLLER**[75] Inventors: **Jiann H. Chen**, Fairport; **Dilip K. Chatterjee**; **Stephen V. Davis**, both of Rochester, all of N.Y.[73] Assignee: **Eastman Kodak Company**, Rochester, N.Y.[21] Appl. No.: **09/035,250**[22] Filed: **Mar. 5, 1998**[51] Int. Cl.<sup>6</sup> ..... **G03G 15/20**[52] U.S. Cl. ..... **399/325; 399/328; 399/333**[58] Field of Search ..... **399/320, 324, 399/325, 328, 330, 331, 333, 335, 339; 430/97, 124**[56] **References Cited**

## U.S. PATENT DOCUMENTS

|           |         |                   |
|-----------|---------|-------------------|
| 3,435,500 | 4/1969  | Aser et al.       |
| 4,659,621 | 4/1987  | Finn et al.       |
| 4,789,565 | 12/1988 | Kon et al.        |
| 4,941,251 | 7/1990  | Sobue et al.      |
| 5,008,221 | 4/1991  | Ketcham.          |
| 5,011,401 | 4/1991  | Sakurai et al.    |
| 5,061,965 | 10/1991 | Ferguson et al.   |
| 5,141,788 | 8/1992  | Badesha et al.    |
| 5,153,660 | 10/1992 | Goto.             |
| 5,166,031 | 11/1992 | Badesha et al.    |
| 5,290,332 | 3/1994  | Chatterjee et al. |

|           |         |                         |
|-----------|---------|-------------------------|
| 5,336,282 | 8/1994  | Ghosh et al. .          |
| 5,358,913 | 10/1994 | Chatterjee et al. .     |
| 5,493,376 | 2/1996  | Heeks .....             |
| 5,543,269 | 8/1996  | Chatterjee et al. .     |
| 5,585,909 | 12/1996 | Behe et al. .           |
| 5,634,184 | 5/1997  | Dalal et al. .....      |
| 5,805,968 | 9/1998  | Chatterjee et al. ..... |
| 5,864,740 | 1/1999  | Heeks et al. .....      |
| 5,871,878 | 2/1999  | Chatterjee et al. ..... |

399/324 X

Primary Examiner—Sandra Brase

Attorney, Agent, or Firm—Raymond L. Owens

[57]

**ABSTRACT**

A fuser for fixing particulate imaging material to a receiver sheet, including a fuser roller and a pressure roller in contact with the fuser roller which engage each other at a fixing nip, wherein pressure is used in fixing the particulate imaging material to the receiver sheet; a supply of offset preventing oil with such offset preventing oil being adapted to react with the zirconia ceramic or its composites to prevent offset of the particulate imaging material; a metering roller in contact with the supply of offset preventing oil for wicking such offset preventing oil onto the surface of the metering roller. The method further includes a donor roller in contact with the metering roller and the fuser roller for receiving offset preventing oil from the metering roller and applying it to the surface of the fuser roller; and one of the rollers forming the fixing nip having a surface formed from zirconia ceramic or its composites which has a hardness greater than 12 GPa and toughness greater than 6 MPa $\sqrt{\text{mm}}$ .

**16 Claims, 1 Drawing Sheet**



**FUSER USING CERAMIC ROLLER****CROSS REFERENCE TO RELATED APPLICATION**

Reference is made to commonly-assigned and concurrently filed U.S. patent application Ser. No. 08/822,163 filed Mar. 21, 1997, entitled "Zirconia Ceramic Roller For Fixing Particulate Imaging Material to a Receiver" by Chatterjee et al and U.S. patent application Ser. No. 08/821,991, filed Mar. 21, 1997, entitled "Toner Offset Preventing Oils for Zirconia Ceramic and Its Composites Rollers" by Chatterjee et al, the teachings of which are incorporated herein by reference.

**FIELD OF THE INVENTION**

The present invention relates to fusers which fix particulate imaging material such as toner to a receiver sheet.

**BACKGROUND OF THE INVENTION**

Electrophotosensitive copiers include a photo conductor with a photoconductive layer with a conductive backing. The photoconductor is transported along an endless path relative to a plurality of work stations, each of which is operative when actuated to perform a work operation on the electrophotosensitive medium. Such stations include a charging station at which a uniform charge is placed on the photoconductive layer, an exposure station at which the charged photoconductive layer is image-wise exposed to actinic radiation from the medium to create an electrostatic image of the medium in the photoconductive layer, a developing station at which the electrostatic image is contacted with finely divided charged toner particles for adhering to the photoconductive layer in a configuration defined by the electrostatic image, a transfer station at which such toner particles are transferred in the image configuration to a receiving surface, and a cleaning station at which residual toner is removed from the photoconductive layer so that it can be reused. The electrostatically held toner image is then adhered to the paper by flowing the toner particles together.

The most common method of adhering the toner to the paper is a combination of heat and pressure to fuse the toner to the paper. The fuser typically includes a pressure roller and a fuser roller and a structure for delivering offset preventing oil to the fuser roller. The fuser roller is heated and the pressure roller may or may not be heated to a temperature less than or equal to the fuser roller so that both heat and pressure are applied to toner particles at the nip between the rollers to fix the toner to a receiver sheet in an image-wise configuration. By convention the fuser roller generally described the roller which comes in contact with the unfused toner and is usually the roller having the higher temperature if there is a temperature differential. The term "fuser" is used herein to identify both the fuser and the pressure roller.

The pressure and fuser rollers performance reliability is one of the most important factors which influences the electrophotographic copier life cycle cost and customer satisfaction. These rollers performance are affected by the ability of the not only the fuser roller, pressure roller, and heating rollers, but also the oiler donor roller and metering rollers to remain free of contamination.

One of the long-standing problems with electrophotographic toner fusing mechanism is the adhesion of the heat-softened toner particles to the surface of the fuser rollers, oiler donor roller, and metering roller as well as to

the receiver, known as "offset" which occurs when the toner-bearing receiver is passed through a fuser. Toner is passed from the fuser to external heater rollers (if present), pressure roller, and oiler donor roller. Toner is passed from the oiler donor roller to the metering roller and from the metering roller to the metering blade. Toner on the metering roller causes streaks while toner on the metering roller causes errors in the oil laydown. Excessive toner build up on heater rolls and both fuser rollers can lead to image defects, jams, and ultimate roller failure. There have been several approaches to decrease the amount of toner offset onto the fuser roller. One approach has been to make the toner-contacting surface of a roller, for example, a fuser roller and/or pressure roller of a non-adhesive (non-stick) material.

5 One known non-adhesive coating for fuser roller comprises fluoropolymer resins, but fluoropolymer resins are non-compliant. It is desirable to have compliant fuser rollers to increase the contact area between a fuser roller and the toner-bearing receiver. However, fuser rollers with a single 10 compliant rubber layer absorb release oils and degrade in a short time leading to wrinkling artifacts, non-uniform nip width and toner offset. To make fluoropolymer resin coated fuser rollers with a compliant layer, U.S. Pat. Nos. 3,435,500 and 4,789,565 disclose a fluoropolymer resin layer sintered to a silicone rubber layer which is adhered to a metal core. In U.S. Pat. No. 4,789,565, an aqueous solution of fluoropolymer resin powder is sintered to the silicone rubber layer. In U.S. Pat. No. 3,435,500, a fluoropolymer resin sleeve is sintered to the silicone rubber layer. Sintering of the 15 fluoropolymer resin layer is usually accomplished by heating the coated fuser rollers to temperatures up to 350° C. Such high temperatures can have a detrimental effect on the silicone rubber layer causing the silicone rubber to smoke or 20 depolymerize, which decreases the durability of the silicone rubbers and the adhesion strength between the silicone rubber layer and the fluoropolymer resin layer. Attempts to 25 avoid the detrimental effect of the high sintering temperatures that have on the silicone rubber layer have been made by using dielectric heating of the fluoropolymer resin layer, 30 for example, see U.S. Pat. Nos. 5,011,401 and 5,153,660. Dielectric heating is, however, complicated and expensive and the fluoropolymer resin layer may still delaminate from the silicone rubber layer when the fuser rollers are used in 35 high pressure fusers. In addition, a fuser roller made with a fluoropolymer resin sleeve layer possess poor abrasion resistance and poor heat resistance.

Again, when a fuser roller becomes contaminated with toner, the contamination can be transferred to a heater roller, thus contributing to the failure. The contamination of the 40 fuser roller can also contribute to the paper jam failure in an electrophotographic engine and it is primarily due largely to the inability of the paper itself to release from the fusing roller. The toner release from the rollers in the electrophotographic engine, which is commonly termed as "offset", is 45 sometimes aided by applying a suitable oil on the roller surface. A probable mechanism for the reduction in offset with oil is that oil flowing into the pores on the surface of the roller material forms a barrier. This barrier is an aid in retarding the offset of contamination. The viscosity of various oils and their molecular structure determine whether the 50 oils will be adsorbed to the roller surfaces. The increase in viscosity makes the displacement of oil from the roller surface more difficult. If a high molecular weight oil is adsorbed on the roller surface, entropy considerations suggest that such oil molecules will have to detach from several 55 sites simultaneously, to regain mobility, making detachment less probable.

The surface energy of the roller material, and its surface morphology can also influence the degree of toner release (offset). Other important material properties such as, wear and abrasion characteristics, thermal conductivity and reactivity or bonding with various functional oils, which are normally used to reduce the offset characteristics can contribute to the choice for suitable heater and pressure roller materials. The commonly used roller material such as elastomers and other experimental roller such as hardcoat anodized rollers, teflon, electroless nickel and electroless nickel impregnated with teflon lack one or more shortcomings in material characteristics described above, and contribute to varying degrees of toner offset.

It has been reported that in order to prevent the offset of toner in a fusing system, attempts have been made to provide a toner release agent also sometimes referred to hereinafter as offset preventing oil, in particular, polydimethylsilicone oil (PDMS) which is applied on the fuser roller to a thickness on the order of about 1  $\mu\text{m}$  to act as a toner release material, these materials possess a relatively low surface energy and have been found to prevent toner from offsetting to the fuser roll surface.

According to prior art techniques, the toner release agents may be applied to fuser roll by several delivery mechanisms including wicking (such as Nomex wick), impregnated webs, or by way of a donor roll.

U.S. Pat. No. 4,659,621 to Finn et al wherein a release agent donor roll is described as having a conformable donor surface comprising the crosslinked product of at least one addition curable vinyl terminated or vinyl pendant PDMS, a silane (Si—H) functional PDMS as crosslinking agent, catalyst and finely divided filler. These donor rolls suffer from roller failure because of the tendency to swell while in contact with the silicone release agent which is absorbed into the silicone rubber. The silicone rubber donor roll no longer can provide a uniform layer of release agent to the fuser roller.

U.S. Pat. No. 5,061,965 to Fergusm et al wherein a release agent donor roll has a base member, an intermediate conformable silicone elastomer layer and an elastomer release agent donor layer comprising poly(vinyldene fluoride-hexafluoropropylene-tetrafluoroethylene) where the vinylidene fluoride is present in an amount <40 mole %, a metal oxide present in an amount sufficient interact with polymeric release agent having functional groups to transport a sufficient amount of the polymeric release agent to provide an interfacial barrier layer between the fusing surface and the toner. This donor roller suffers from the oil wetting capability between the nonfunctional PDMS release agent and the nonreactive donor roller surface since the invention counts on the polymeric release agent having functional groups to react with the metal oxide which is dispersed into the fluoroelastomer layer.

U.S. Pat. No. 5,141,788 and U.S. Pat. No. 5,166,031 to Santokh Badesha wherein a release agent donor roll comprising a supporting substrate having an outer layer of a surface grafted or volume grafted polyorganosiloxane formed by dehydrofluorination of said fluoroelastomer by a nucleophilic dehydrofluorinating agent, followed by addition polymerization by the addition of an alkene functionalized polyorganosiloxane and a polymerization initiator. Fabricated donor rolls used for supplying conventional silicone oil release agent showed 4.3 million copies without failure. Although these rolls provide long life, non-oil swelling, and can also be used with non-functional PDMS release agent, the manufacturing of such a donor roll is tedious, inefficient, and expensive.

#### SUMMARY OF THE INVENTION

It is an object of the present invention to provide a fuser which eliminate the problems discussed above.

This object is achieved in a A fuser for fixing particulate imaging material to a receiver sheet, comprising:

- (a) a fuser roller and a pressure roller in contact with the fuser roller which engage each other at a fixing nip, wherein pressure is used in fixing the particulate imaging material to the receiver sheet;
- (b) a supply of offset preventing oil with such offset preventing oil being adapted to react with the zirconia ceramic or its composites to prevent offset of the particulate imaging material;
- (c) a metering roller in contact with the supply of offset preventing oil for wicking such offset preventing oil onto the surface of the metering roller;
- (d) a donor roller in contact with the metering roller and the fuser roller for receiving offset preventing oil from the metering roller and applying it to the surface of the fuser roller; and
- (e) one of the rollers forming the fixing nip having a surface formed from zirconia ceramic or its composites which has a hardness greater than 12 GPa and toughness greater than 6 MPa $\sqrt{\text{mm}}$ .

Another object of the present invention is to uniformly apply offset preventing oil to the donor roller. This can be achieved by forming the metering roller of zirconia ceramic or its composites.

Ceramic roller used as fusers in accordance with the present invention have increased hardness, toughness and are chemically resistant to corrosion. When used in electro-photographic apparatus, fusing or fixing is improved and jamming of receiver sheets is reduced. Fuser roller life is improved because of the high wear and abrasion resistant properties of zirconia and its composites.

The unusually high wear abrasion and corrosion resistance of these materials make them particularly suitable for roller material in an electrophotographic apparatus. In the charging section of electrophotographic copiers, ozone may be generated which is a highly corrosive gas. Materials in accordance with the present invention are resistant to attack by ozone.

In accordance with the present invention when the donor roller or the metering roller is formed of zirconia ceramic or its composites, such a roller would have a long life, and of course would not swell when offset preventing oil is applied to the roller. Offset preventing oil in accordance with the present invention when applied to a zirconia ceramic or its composites roller has the following advantages:

1. 0% oil swell
2. good oil uniformity
3. steady oil rate
4. excellent wear rate
5. no oil streaks, wings or slippage

#### BRIEF DESCRIPTION OF THE DRAWINGS

The FIGURE is a schematic front cross-sectional view of a fuser in accordance with the present invention.

#### DETAILED DESCRIPTION OF THE PREFERRED EMBODIMENTS

Referring now to the FIGURE a fuser is shown which includes a fuser roller 20 and an elastomeric pressure roller 28 which form a nip 30. A supply of offset preventing oil 33

is shown provided in a oil reservoir 34. The fuser roller 20 can be made of zirconia ceramic and its composites as will be discussed later. Particulate imaging material 40 disposed on a receiver 42 is fused into the receiver 42 at the nip 30 by the application of heat and pressure. As shown a heating lamp 44 is connected to a control circuit 46. The heating lamp 44 is well known to those skilled in the art is provided inside the core of the fuser roller 20. Alternatively, the fuser may be externally heated by a heated roller riding along the fuser roller 20. This external heated may replace or merely assist the internal lamp. It will be understood depending on the particulate imaging material 40 that is used that only pressure need be applied to fuse particulate imaging material 40 into the receiver 42. A wicking device 32 shown in the form of a wick 36, absorbs the offset preventing oil 33 and is contacted by a metering roller 48 intermediate between the fuser roller 20 and the metering roller 48 is a donor roller 50. The donor roller 50 delivers offset preventing oil 33 to the particulate imaging material 40 to the receiver 42. A continuous supply of offset preventing oil 33 must be used which is approximately 1 to 20 mg per receiver 42, on which particulate imaging material 40 is fixed. This offset preventing oil will be discussed in much more detail later.

It is not practical to have two rollers made of zirconia ceramic or its composites in contact with each other as no appreciable nipwidth could be obtained and the material could be worn more rapidly by itself. In accordance with the present invention, there are several possibilities, the fuser roller 20 itself can have its surface formed of  $ZrO_2$  or  $ZrO_2-Al_2O_3$  (zirconia composite). In such a situation, the metering roller 48 can also be formed of  $ZrO_2$  or  $ZrO_2-Al_2O_3$  (zirconia composite). As another embodiment, only the donor roller 50 can be formed of  $ZrO_2$  or  $ZrO_2-Al_2O_3$  (zirconia composite). The rollers which are not formed from  $ZrO_2$  or  $ZrO_2-Al_2O_3$  (zirconia composite) are preferably made from a compliant material such as silicone- or fluor elastomer or foam. When a roller surface is made of or zirconia composite more thermal conductivity than zirconia and so it is used to provide rollers which transfer heat. On the other hand, zirconia is a poor heat conductor and so after it is heated it will maintain a given temperature for a longer time.

Zirconia has the chemical composition of  $ZrO_2$  and with a predominately tetragonal crystal structure. The composites of zirconia can take many forms, however, in accordance with this invention that term shall mean alumina composites ( $ZrO_2-Al_2O_3$ ), which will be discussed in more detail later. These materials, because of its specific crystallographic nature, which will be described later, have high hardness, and unusually high fracture toughness for ceramics. The zirconia ceramic and its composites materials have a hardness greater than 12 GPa and toughness greater than 6 MPa  $\sqrt{mm}$ . Sometimes it is desirable to heat the roller and in such a case, the fuser roller 20 would be formed with a cavity and a heated lamp can be provided inside of either or both of the fuser rollers 20 and pressure roller 28. The pressure rollers 28 are formed of different compliant materials such as silicon or fluorocarbon.

Zirconia ceramic, particularly yttria doped tetragonal zirconia polycrystals (Y-TZP) and its composites such as  $ZrO_2-Al_2O_3$  are known to posses high wear and abrasion resistance. Tetragonal zirconia also has high hardness and high fracture in toughness. It is also known that surface energy of the zirconia ceramics and its composites can be modified by changing the oxidation states of the materials. It is further known that infrared energy can be successfully utilized to modify both the surface morphology and surface energy of zirconia ceramics and its composites.

Pure zirconia powder is alloyed with stabilizing agents as described by Chatterjee et al in commonly-assigned U.S. Pat. No. 5,358,913 to form zirconia alloy powder which has predominately a tetragonal crystal structure. One such example of such powder is yttria stabilized tetragonal zirconia polycrystals (Y-TZP). Y-TZP can also be mixed with other ceramic powders to form composites. One example of such a composites are zirconia-alumina composites, where the alumina concentration can vary from 0.1 to 50 weight percent. It has been found preferable to use a weight percentage of alumina of about 20 percent

The powders described above form the starting materials for the formation and manufacture of rollers for the electrophotographic engine. The rollers can be manufactured either by cold pressing or cold isostatic pressing or by injection molding and sintering. The various procedures for manufacturing rollers using ceramic materials, particularly for Y-TZP and its composites are disclosed by Ghosh et al in commonly-assigned U.S. Pat. No. 5,336,282 and Chatterjee et al in commonly-assigned U.S. patent application Ser. No. 08/740,452 filed Oct. 28, 1996.

Yttria-doped tetragonal zirconia polycrystal (Y-TZP) ceramic materials offer many advantages over conventional materials, including many other ceramics. Y-TZP is one of the toughest ceramics. The toughness is achieved at the expense of hardness and strength. Tetragonal zirconia alloy-alumina composite, that is, the product of sintering a particulate mixture of zirconia alloy and alumina, is another tough and relatively softer structural ceramic composite.

The zirconium oxide alloy is made essentially of zirconium oxide and a secondary oxide selected from the group consisting of  $MgO$ ,  $CaO$ ,  $Y_2O_3$ ,  $Sc_2O_3$ ,  $Ce_2O_3$  and rare earth oxides. Moreover, the zirconium oxide alloy has a concentration of the secondary oxide of, in the case of  $Y_2O_3$ , about 0.5 to about 5 mole percent; in the case of  $MgO$ , about 0.1 to about 1.0 mole percent; in the case of  $CeO_2$ , about 0.5 to about 15 mole percent; in the case of  $Sc_2O_3$ , about 0.5 to about 7.0 mole percent and in the case of  $CaO$  from about 0.5 to about 5 mole percent, relative to the total of the zirconium oxide alloy. A mold is provided for receiving and processing the zirconia alloy ceramic powder or its composites. The ceramic powder is then compacted by cold isostatic pressing in the mold provided to form a ceramic blank or billet. The ceramic billet is then shaped or green-machined so as to form near net-shaped roller. The term "green" refers to the ceramic roller before sintering. After the initial shaping, the green rollers are sintered thereby forming sintered net-shaped ceramic rollers. The ceramic rollers for the electrophotographic apparatus described above, are then further machined or shaped until finished rollers are formed.

The preferred ceramic composite powder mixture in the method of making zirconia-alumina ceramic composites of the invention includes a particulate zirconia alloy and a particulate alumina made by mixing  $ZrO_2$  and additional "secondary oxide" selected from:  $MgO$ ,  $CaO$ ,  $Y_2O_3$ ,  $Sc_2O_3$  and  $Ce_2O_3$  and other rare earth oxides (also referred to herein as "Mg—Ca—Y—Sc—rare earth oxides") and then with  $Al_2O_3$ . Zirconia alloys useful in the methods of the invention have a metastable tetragonal crystal structure in the temperature and pressure ranges at which the ceramic article produced will be used. For example, at temperatures up to about 200° C. and pressures up to about 1000 MPa, zirconia alloys having, wherein zirconium oxide alloy has a concentration of the secondary oxide of, in the case of  $Y_2O_3$ , about 0.5 to about 5 mole percent; in the case of  $MgO$ , about 0.1 to about 1.0 mole percent, in the case of  $Ce_2O_3$ , about 0.5

to about 15 mole percent, in the case of  $\text{Sc}_2\text{O}_3$ , about 0.5 to about 7.0 mole percent and in the case of  $\text{CaO}$  from about 0.5 to about 5 mole percent, relative to the total of the zirconium oxide alloy, the compacting further comprising forming a blank and then sintering, exhibit a tetragonal structure. Preferred oxides for alloying with zirconia are  $\text{Y}_2\text{O}_3$ ,  $\text{MgO}$ ,  $\text{CaO}$ ,  $\text{Ce}_2\text{O}_3$  and combinations of these oxides. It is preferred that the zirconia powder have high purity, greater than about 99.9 percent. Specific examples of useful zirconia alloys include: tetragonal structure zirconia alloys having from about 2 to about 5 mole percent  $\text{Y}_2\text{O}_3$ , or more preferably about 3 mole percent  $\text{Y}_2\text{O}_3$ . Examples of tetragonal structure zirconia alloys are disclosed in U.S. Pat. No. 5,290,332. Such zirconia alloys are described in that patent as being useful to provide a ceramic roller.

The grain and agglomeration sizes and distributions, moisture contents, and binders (if any) can be varied in both the alumina and the zirconia alloy, in a manner known to those skilled in the art. "Grain" is defined as an individual crystal, which may be within a particle, having a spatial orientation that is distinct from that of adjacent grains. "Agglomerate" is defined as an aggregation of individual particles, each of which may comprise multiple grains. In a particular embodiment of the invention, the grain and agglomeration sizes and distributions, and moisture contents of the alumina and the zirconia alloy are substantially the same and are selected as if the zirconia alloy was not going to be mixed with the alumina, that is in a manner known to the art to be suitable for the preparation of a zirconia alloy article.

An example of convenient particulate characteristics for a particular embodiment of the invention is the following. Purity of  $\text{ZrO}_2$  is preferably well controlled at 99.9 to 99.99 percent, that is, impurities are no more than about 0.1 to 0.01 percent. The grain size is from about 0.1 micrometers to about 0.6 micrometers. The average grain size is 0.3 micrometers. The distribution of grain sizes is: 5-15 percent less than 0.1 micrometers, 40-60 percent less than 0.3 micrometers, and 85-95 percent less than 0.6 micrometers. The surface area of each individual grain ranges from about 10 to about 15  $\text{m}^2/\text{gram}$  or is preferably 14  $\text{m}^2/\text{gram}$ . Agglomerate size is from about 30 to about 60 micrometers and average agglomerate size is: 40-60 micrometers. Moisture content is about 0.2 to 1.0 percent by volume of blank and is preferably 0.5 percent. The mixture of particulate is compacted in the presence of an organic binder.

Binders such as gelatin or polyethylene glycol(PEG) or acrylic or polyvinyl ionomer or more preferably polyvinyl alcohol, are added to and mixed with the particulate mixture Y-TZP, or a composite mixture of Y-TZP and alumina. This can be achieved preferably by spray drying or ball milling prior to placement of the mixture in a compacting device.

The particulate mixture of zirconia alloy and/or zirconia-alumina ceramic composite is compacted; heated to a temperature range at which sintering will occur; sintered, that is, maintained at that temperature range for a period of time; and then cooled. During sintering, individual particles join with each other and transform from "green preform" to a dense article. This densification is achieved by diffusion controlled process. In an alternate embodiment, during all or part of sintering, the particulate mixture compact or the "green preform" is kept in contact with a preselected dopant, as discussed below in detail, to further improve the surface properties of the sintered articles.

Preferably, the powder mixture is cold compacted to provide a "green preform", which has a "green" density that

is substantially less than the final sintered density of the ceramic roller of electrophotographic apparatus. It is preferred that the green density be between about 40 and about 65 percent of the final sintered density, or more preferably be about 60 percent of the final sintered density.

Then the green rollers are sintered to full density using preferably sintering schedules described in U.S. Pat. Nos. 5,336,282 and 5,358,913, hereby incorporated hereby by reference, and final precision machining of the final sintered rollers were made to tight tolerances to produce the rollers of electrophotographic apparatus of the invention using diamond tools. Near net-shaped green preforms produced either by dry pressing or by injection molding, respectively, did not warrant green machining to generate net-shaped rollers after sintering. Only billets or blanks of zirconia ceramic or its composites produced by cold isostatic pressing needed green machining before sintering. The near-net-shaped green preform produced by injection molding needed an additional step called "debinding" wherein excess organic binders are removed by heating the preforms at around 250° C. for about 12 hours prior to sintering.

In an alternate embodiment of the sintering process, the dopant oxide selected from  $\text{MgO}$ ,  $\text{FeO}$ ,  $\text{ZnO}$ ,  $\text{CoO}$ ,  $\text{NiO}$ , and  $\text{MnO}$ , and combination thereof, is in contact with the blank. It is preferred that the sintering result in a ceramic and/or composite rollers having a "full" or nearly theoretical density, and it is more preferred that the density of the ceramic rollers be from about 99.5 to about 99.9 percent of theoretical density. Sintering is conducted in air or other oxygen containing atmosphere.

Sintering can be performed at atmospheric pressure or alternatively a higher pressure, such as that used in hot isostatic pressing can be used during all or part of the sintering to reduce porosity. The sintering is continued for a sufficient time period for the case of the article being sintered to reach a thermodynamic equilibrium structure. An example of a useful range of elevated sintering pressures is from about 69 MPa to about 207 MPa, or more preferably about 100 to 103 MPa.

The toners used in the working and comparative examples of this invention are 100 percent unfused EK1580 toner (Eastman Kodak Company, Rochester, N.Y.). The off-line testing of the roller material is carried out both in the "dry" condition and also in the "wet" condition, where the roller materials, in the form of a plate are treated with offset preventing oils. The experimental set-up for the off-line test, wherein a heated bed on which the roller materials of interest were placed. An inch square piece of paper with 100% unfused toner laydown was then placed in intimate contact with the roller materials in the specific case, Y-TZP and its composites with alumina. To ensure the intimate contact a clamp was used. The bed of the tester is heated to predetermined fusing temperatures and a thermocouple (not shown) registers this temperature. Two temperatures, 165° C. and 190° C. were used. A pressure application device set for 80 pounds per square inch was then locked in place over the roller material/toner/paper sandwich. The pressure was applied for such off-line testing from a minimum of 30 seconds to a maximum, in most cases of 20 minutes. The release characteristics were evaluated by visual inspection of the fused paper.

The ceramic rollers of this invention was also irradiated with infrared energy specifically with a Nd-YAG laser of 1.06  $\mu\text{m}$  wavelength operated at various conditions. Laser assisted irradiation of these materials causes a surface chemical composition change of the ceramic materials used

in this invention. As disclosed by Chatterjee et al in commonly-assigned U.S. Pat. No. 5,543,269 laser induced surface, that the chemical composition change is associated with surface energy change and it is believed in the specific case of the present invention that reactivity of the particulate imaging material with the roller material are modified through the change in its surface energy. However, laser irradiation of materials can be a source of degradation of surface morphology. The rough surface morphology can cause toner offset. Hence, laser irradiation parameters have to be selected judiciously to take advantage of the surface energy reduction.

Quite unexpectedly it has been found that certain offset preventing oils react with zirconia ceramic or its composites to prevent offset. In accordance with the present invention, it has been found to be highly desirable to first react the surface of the fusing roller with these offset preventing oils. Thereafter, during the process of fixing particulate imaging material images these offset preventing oils can be wicked onto the surface of the fuser roller **20** during the process of fixing particulate imaging material. The following is a discussion of the different offset preventing oils which can be used with treated and untreated rollers which have their surfaces formed of zircon ceramic or its composites.

The following summary shows the types of offset preventing oil that will be effective with treated and untreated zirconia and treated and untreated zirconia composites.

| Roller                                                | Zirconia ( $\text{ZrO}_2$ )                                                                        | Zirconia Composites ( $\text{ZrO}_2\text{--Al}_2\text{O}_3$ )                                      |
|-------------------------------------------------------|----------------------------------------------------------------------------------------------------|----------------------------------------------------------------------------------------------------|
| Two Material Processing for Each Material             | 1) Untreated<br>2) Treated with IR Laser                                                           | 1) Untreated<br>2) Treated with IR Laser                                                           |
| Three Oils (for untreated materials) for release      | 1) Non functional                                                                                  | 1) Non-functional                                                                                  |
|                                                       | $\begin{array}{c} \text{CH}_3 \\   \\ \text{CH}_3\text{---Si---O} \\   \\ \text{CH}_3 \end{array}$ | $\begin{array}{c} \text{CH}_3 \\   \\ \text{CH}_3\text{---Si---O} \\   \\ \text{CH}_3 \end{array}$ |
|                                                       | 2) Silane<br>$\text{H---Si---H}$                                                                   | 2) Silane<br>$\text{H---Si---H}$                                                                   |
|                                                       | 3) Amino<br>$\text{H}_2\text{N---CH}_2\text{CH}_2\text{CH}_2$                                      | 3) Amino<br>$\text{H}_2\text{N---CH}_2\text{CH}_2\text{CH}_2$                                      |
| Two Oils (for IR Laser Treated Materials) for release | 1) Silane<br>$\text{H---Si---H}$                                                                   | 1) Silane<br>$\text{H---Si---H}$                                                                   |
|                                                       | 2) Amino<br>$\text{H}_2\text{N---CH}_2\text{CH}_2\text{CH}_2$                                      | 2) Amino<br>$\text{H}_2\text{N---CH}_2\text{CH}_2\text{CH}_2$                                      |

TABLE I

## Laser Irradiation Conditions

Nd:YAG Laser:Wavelength = 1.06  $\mu\text{m}$   
Pulse Frequency = 1 KHz  
Bite Size = 0.05209 mm  
Peak Power = 6,000–67,000 Watts  
Current = 18–28 amps  
Energy = 0.6 mJ to 5.2 mJ  
Energy Density = 7  $\text{J/cm}^2$  to 66  $\text{J/cm}^2$

The rollers which use zirconia ceramic or its composites produced in accordance with the present invention are useful in electrophotographic copying machines to fuse heat-softenable toner to a substrate. This is accomplished by contacting a receiver, such as a sheet of a paper, to which toner particle are electrostatically attached in an imagewise fashion, with such a fuser roller **20**. Such contact is main-

tained at a temperature and pressure sufficient to fuse or fix the toner to the receiver. Because these members are so durable they can be cleaned using a blade pad, roller or brush during use. The following is a discussion of offset preventing oils that can be used with any of the untreated ceramic rollers and with a treated (irradiated) ceramic rollers that can be used in accordance with this invention. It has been found that in either case offset preventing oils that are effective have compounds having functional groups selected from the group including  $-\text{CH}_2\text{---CH}_2\text{---CH}_2\text{---NH}_2$  and



When untreated ceramic rollers are used, the offset preventing oil has functional groups selected from the groups consisting of  $-\text{CH}_2\text{---CH}_2\text{---CH}_2\text{---NH}_2$ ,



When treated ceramic rollers are used the offset preventing oil has functional groups selected from the groups consisting of  $-\text{CH}_2\text{---CH}_2\text{---CH}_2\text{---NH}_2$  and



Another aspect of the change in the reactivity of the toner particles with some functional offset preventing oils. As described hereinafter that the reactivity of toner particles with the roller materials is hindered by formation of some sort of barriers caused by the absorption of offset preventing oils into the pores of the roller materials. The rheological property, such as viscosity and the chemical property, such as molecular weight of the offset preventing oils will greatly influence the barrier formation between the toner particles and the roller materials.

Chemical structure of functional polydimethyl siloxane and non-functional polydimethyl siloxane (PDMS) which will be discussed as follows:

## 1. Non-functional PDMS



## 2. Mercapto functional PDMS



-continued

## 3. Silane functional PDMS



wherein

m, n:  $1\% \leq m \leq 99\%$  $1\% \leq n \leq 99\%$  $m + n = 100\%$ 

## 4. Amino functional PDMS



wherein

A: is  $-\text{CH}_2-\text{CH}_2-\text{CH}_2-\text{NH}_2$  $50 \leq n \leq 1000$ 

R: is an alkyl or aryl group

Examples (for laser irradiated zirconia ceramic or its composites rollers)

The affinity of the functional offset preventing oil of this invention to laser treated ceramic fuser roller **20** surface in the process of the present invention can be assessed from the results of applying functional polydimethyl siloxane release offset preventing oil to a fuser roller **20** surface (Heated Roll) comprising, for example, a 18 amp zirconia ceramic or its composites samples laser treated using 18 amps incubating the samples for overnight (12 hrs) at 170° C. in contact with the functional PDMS, and then subjecting the ceramic surface to soak in DCM (dichloromethane) for one hour, removed and wiped to clean unreacted functional offset preventing oil. Qualitative measurements of the attachment of the polydimethyl siloxane to the surface of the laser treated ceramic were carried out by the off-line toner combination unit. The off-line test for toner contamination is a heated bed on which the ceramic samples are placed. A 1" square piece of paper with 100% unfused EK1580 toner is put in contact with the ceramic samples which are cut into a 1" squares. The sandwich is then heated to a temperature of 175° C. A pressure roller **28** set for 80 psi is then locked in place over the sample for 20 minutes. The test forms a nip under pressure and the interaction between the toned paper and the ceramic sample in the nip area is examined using an optical microscope. The toner release performance of the ceramic sample is assessed by the amount of toner (offset) on the surface of the ceramic sample.

Three major types of functional offset preventing oil (silane functional offset preventing oil, amino functional offset preventing oil, and mercapto functional offset preventing oil) were used in the test. In addition, the non-functional offset preventing oil and no offset preventing oil also were used as controls.

Specific examples of commercially available functionalized polydimethylsiloxanes of utility in this invention include:

- 1) organohydrosiloxane copolymers such as
  - (a) PS 123, (30-35%) methylhydro-(65-70%) dimethylsiloxane
  - (b) PS 124.5, (3-4%) methylhydro-(96-99%) dimethylsiloxane which are available from United Chemical, Inc.
- 2) aminopropyldimethyl terminated polydimethylsiloxane Xerox 5090 fuser agent which is available from Xerox
- 3) mercapto functional polydimethylsiloxane Xerox 5090 fuser agent which is available from Xerox

4) non-functional polydimethylsiloxane, trimethylsiloxane terminated DC-200, 350 Cts which is available from Dow Corning

Table II below shows the results obtained from the examples.

TABLE II

| Zirconia Ceramic and its Composite Materials* |                        | Siloxane        | Organopoly-Group   | Functional Offset | Oil Reactivity |
|-----------------------------------------------|------------------------|-----------------|--------------------|-------------------|----------------|
| 10                                            | 18 amp                 | None            | None               | Heavy             | No             |
| 15                                            | 18 amp                 | DC-200, 350 Cts | trimethyl-siloxane | Heavy             | No             |
| 18 amp                                        | Xerox 5090 fuser agent | mercapto-propyl | Heavy              | No                |                |
| 18 amp                                        | PS-123                 | hydro-silane    | None               | Yes               |                |
| 18 amp                                        | PS-124.5               | hydro-silane    | None               | Yes               |                |
| 18 amp                                        | Xerox 5090 fuser agent | amino-propyl    | Slight             | Yes               |                |
| 20                                            | 24 amp                 | PS-124.5        | hydro-silane       | Heavy             | No             |
| 24 amp                                        | Xerox 5090 fuser agent | amino-propyl    | Heavy              | No                |                |
| 24 amp                                        | Xerox 5090 fuser agent | mercapto-propyl | Heavy              | No                |                |

\*Laser treated using conditions described in Table I.

For a surface (ceramic fusing member) reacted and covered with functional polydimethylsiloxane, the toner offset should be zero or close to zero (slight offset). Referring to 30 Table II, the non-functionalized polydimethylsiloxane DC-200 or no offset preventing oil used provide no offset preventing oil coverage on the ceramic samples. Use of the Si—H functionalized polydimethylsiloxane PS-123, and PS-124.5 provide superior toner release properties. Use of 35 the aminopropylsiloxane functionalized polydimethylsiloxane Xerox 5090 fuser agent also provides the offset preventing oil coverage, but this functional offset preventing oil suffers slight offset. Thus, results as good or better than those with the non-functionalized polydimethylsiloxane or no 40 polydimethylsiloxane can be obtained by use of a functional polydimethylsiloxane comprising a Si—H functionalized PDMS or aminopropyl functionalized PDMS with the zirconia ceramic and its composites laser treated following the conditions described in Table I in accordance with the 45 invention.

Referring to Table II, the use of a zirconia ceramic and its composites laser treated using 24 amps following the conditions described in Table I with the functionalized PDMS (see C-4, C-5, C-6) did not provide any offset preventing oil 50 coverage on the ceramic samples. The laser operating conditions for treatment of zirconia ceramic and its composite samples are important.

The high affinity of Si—H functionalized and aminopropyl 55 functionalized organopolysiloxane with the 18 amp ceramic compound for donor roller **50** and metering roller **48** surface provides excellent release of fused toner image. Use of this surface as a donor roll or metering roll to deliver steady and uniform oil rate in a fusing process provides a highly effective way of meeting the need for excellent release 60 characteristics without excessive wear of the heat roll surface.

Examples (untreated zirconia ceramic or composite rollers)

The affinity of functional offset preventing oil of this 65 invention to untreated (non-laser irradiated) ceramic fuser roller **20** surface in the process of this invention can be assessed from the results of applying functional polydimethylsiloxane release offset preventing oil to a donor roller **50** or

metering roller **48** surface (Heated Roll) comprising an untreated ceramic  $\text{ZrO}_2$ . The samples were treated and tested similar to the previous examples.

Referring to Table III below, the mercapto functionalized PDMS and no offset preventing oil provide no protection on the surface of the ceramic sample. Use of Si—H functionalized PDMS PS-123, PS-124.5, aminopropyl functionalized PDMS and non-functionalized PDMS provide superior toner release property on the untreated  $\text{ZrO}_2$  ceramic materials. Use of this surface in a fusing process to deliver a steady and uniform oil rate provides a highly effective way of meeting the need for excellent release characteristics without excessive wear of the fuser roller **20** and without encountering the problems of odor and toxicity associated with use of mercapto-functional polydimethylsiloxanes.

Table III below shows the results obtained from the examples of untreated zirconia ceramic or its composites.

TABLE III

| Zirconia Ceramic and its Composite Materials | Organopoly-siloxane                   | Toner Offset | Oil Reactivity |
|----------------------------------------------|---------------------------------------|--------------|----------------|
| untreated                                    | None                                  | Heavy        | No             |
| untreated                                    | Xerox 5090 fuser agent                | Heavy        | No             |
| untreated                                    | Mercapto-functionalize                |              |                |
| untreated                                    | PS-123 Si-H                           | None         | Yes            |
| untreated                                    | PS-124.5 Si-H                         | Slight       | Yes            |
| untreated                                    | functionalized                        |              |                |
| untreated                                    | Xerox 5090 Amino-function fuser agent | Slight       | Yes            |
| untreated                                    | DC-200                                | Slight       | Yes            |

Briefly reviewing the FIGURE, in the situation where the fuser roller **20** is made of zirconia ceramic or its composites then the pressure roller **28** and the donor roller **50** should be formed from compliant material. The reason for this is that it is not effective to have two ceramic rollers in contact with each other since they are formed of very hard material and will not deform to form an appropriate nip. In the situation where the pressure roller **28** is made of zirconia ceramic or its composites then the fuser roller **20** must be compliant and the donor roller **50** can be formed of zirconia ceramic or its composites. Alternatively, it can be desirable to form only the metering roller **48** of zirconia ceramic or its composites. In this case the donor roller **50** must be compliant and the fuser roller **20** could be formed from zirconia ceramic or its composites. When only the metering roller **48** is made from zirconia ceramic or its composites such roller can provide a uniform distribution of offset preventing oil to the donor roller **50**.

The invention has been described in detail with particular reference to certain preferred embodiments thereof, but it will be understood that variations and modifications can be effected within the spirit and scope of the invention.

## PARTS LIST

- 20** fusing roller
- 22** heater roller
- 24** heater roller
- 28** pressure roller
- 30** nip
- 33** offset preventing oil
- 34** oil reservoir
- 36** wick
- 40** particulate imaging material

- 42** receiver
- 44** heating lamp
- 46** control circuit
- 48** metering roller
- 50** donor roller

What is claimed is:

**1.** A fuser for fixing particulate imaging material to a receiver sheet, comprising:

- (a) a fuser roller and a pressure roller in contact with the fuser roller which engage each other at a fixing nip, wherein pressure is used in fixing the particulate imaging material to the receiver sheet;
- (b) a supply of offset preventing oil with such offset preventing oil being adapted to react with a zirconia ceramic or its composites to prevent offset of the particulate imaging material;
- (c) a metering roller in contact with the supply of offset preventing oil for wicking such offset preventing oil onto the surface of the metering roller;
- (d) a donor roller in contact with the metering roller and the fuser roller for receiving offset preventing oil from the metering roller and applying it to the surface of the fuser roller; and
- (e) wherein the surface of the donor roller is formed from zirconia ceramic or its composites which has a hardness greater than 12 GPa and toughness greater than 6 MPa  $\sqrt{\text{mm}}$ .

**2.** The fuser of claim **1** wherein the surface of the metering roller and the surface of the fuser roller are formed from zirconia ceramic or its composites, and wherein the donor roller is formed from a compliant material.

**3.** The fuser of claim **1** wherein the offset preventing oil includes compounds having functional groups selected from the groups consisting of  $-\text{CH}_2-\text{CH}_2-\text{CH}_2-\text{NH}_2$ ,



**4.** The fuser of claim **1** wherein the offset preventing oil has been treated with IR laser light to change the surface energy of the zirconia ceramic or its composite includes compounds having functional groups selected from the groups consisting of  $-\text{CH}_2-\text{CH}_2-\text{CH}_2-\text{NH}_2$  and



**5.** The fuser of claim **4** wherein the offset preventing oils are selected from the group consisting of:



**A:** is  $-\text{CH}_2-\text{CH}_2-\text{CH}_2\text{NH}_2$

**n:**  $50 \leq n \leq 1000$

15

R is an alkyl or aryl group



wherein

m,n:  $1\% \leq m \leq 99\%$  $1\% \leq n \leq 99\%$  $m+n=100\%$ ; andwhere n:  $50 \leq n \leq 1000$ .

6. The fuser of claim 4 wherein the offset preventing oil includes compounds having functional groups selected from the groups consisting of:



wherein

m,n:  $1\% \leq m \leq 99\%$  $1\% \leq n \leq 99\%$  $m+n=100\%$ ; andA is  $-\text{CH}_2-\text{CH}_2-\text{CH}_2-\text{NH}_2$ n:  $50 \leq n \leq 1000$ 

R is an alkyl or aryl group.

7. The fuser of claim 4, wherein the offset preventing oil was reacted with the zirconia ceramic or its composites prior to fixing the particulate imaging material and which prevents offset of the particulate imaging material.

8. A fuser for fixing particulate imaging material to a receiver sheet, comprising:

(a) a fuser roller and a pressure roller in contact with the fuser roller which engage each other at a fixing nip, wherein pressure is used in fixing the particulate imaging material to the receiver sheet;

(b) means for applying heat to the fuser roller for use in fixing the particulate imaging material to the receiver sheet;

(c) a supply of offset preventing oil with such offset preventing oil being adapted to react with a zirconia ceramic or its composites to prevent offset of the particulate imaging material;

(d) a metering roller in contact with the supply of offset preventing oil for wicking such offset preventing oil onto the surface of the metering roller;

(e) a donor roller in contact with the metering roller and the fuser roller for receiving offset preventing oil from

16

the metering roller and applying it to the surface of the fuser roller; and

(f) wherein the surface of the donor roller is formed from zirconia ceramic or its composites which has a hardness greater than 12 GPa and toughness greater than 6 MPa  $\sqrt{\text{mm}}$ .

9. The fuser of claim 8 wherein the offset preventing oil includes compounds having functional groups selected from the groups consisting of  $-\text{CH}_2-\text{CH}_2-\text{CH}_2-\text{NH}_2$ ,



10. The fuser of claim 8 wherein the offset preventing oil has been treated with IR laser light to change the surface energy of the zirconia ceramic or its composite includes compounds having functional groups selected from the groups consisting of  $-\text{CH}_2-\text{CH}_2-\text{CH}_2-\text{NH}_2$  and



11. The fuser of claim 10 wherein the offset preventing oils are selected from the group consisting of:



40 A: is  $-\text{CH}_2-\text{CH}_2-\text{CH}_2-\text{NH}_2$

n:  $50 \leq n \leq 1000$ 

R is an alkyl or aryl group



wherein

m,n:  $1\% \leq m \leq 99\%$  $1\% \leq n \leq 99\%$  $m+n=100\%$ ; andwhere n:  $50 \leq n \leq 1000$ .

12. The fuser of claim 10 wherein the offset preventing oil includes compounds having functional groups selected from the groups consisting of:



wherein

m,n:  $1\% \leq m \leq 99\%$   
 $1\% \leq n \leq 99\%$   
 $m+n=100\%$ ; and



A is  $-\text{CH}_2-\text{CH}_2-\text{CH}_2-\text{NH}_2$

n:  $50 \leq n \leq 1000$

R is an alkyl or aryl group.

13. The fuser of claim 10, wherein the offset preventing oil was reacted with the zirconia ceramic or its composites prior to fixing the particulate imaging material and which prevents offset of the particulate imaging material.

14. A fuser for fixing particulate imaging material to a receiver sheet, comprising:

- (a) a fuser roller and a pressure roller in contact with the fuser roller which engage each other at a fixing nip, wherein pressure is used in fixing the particulate imaging material to the receiver sheet;
- (b) a supply of offset preventing oil with such offset preventing oil being adapted to react with a zirconia ceramic or its composites to prevent offset of the particulate imaging material;
- (c) a metering roller in contact with the supply of offset preventing oil for wicking such offset preventing oil onto the surface of the metering roller;
- (d) a donor roller in contact with the metering roller and the fuser roller for receiving offset preventing oil from the metering roller and applying it to the surface of the fuser roller; and
- (e) the metering roller having a surface formed from zirconia ceramic or its composites which has a hardness greater than 12 GPa and toughness greater than  $6 \text{ MPa}^{\sqrt{\text{mm}}}$ .

15. A fuser for fixing particulate imaging material to a receiver sheet, comprising:

- (a) a fuser roller and a pressure roller in contact with the fuser roller which engage each other at a fixing nip,

wherein pressure is used in fixing the particulate imaging material to the receiver sheet;

- (b) a supply of offset preventing oil with such offset preventing oil being adapted to react with a zirconia ceramic or its composites to prevent offset of the particulate imaging material;
- (c) a metering roller in contact with the supply of offset preventing oil for wicking such offset preventing oil onto the surface of the metering roller;
- (d) a donor roller in contact with the metering roller and the fuser roller for receiving offset preventing oil from the metering roller and applying it to the surface of the fuser roller; and
- (e) wherein the surface of the metering roller and fuser roller are formed from zirconia ceramic or its composites which has a hardness greater than 12 GPa and toughness greater than  $6 \text{ MPa}^{\sqrt{\text{mm}}}$  and wherein the donor roller is formed from a compliant material.

16. A fuser for fixing particulate imaging material to a receiver sheet, comprising:

- (a) a fuser roller and a pressure roller in contact with the fuser roller which engage each other at a fixing nip, wherein pressure is used in fixing the particulate imaging material to the receiver sheet;
- (b) means for applying heat to the fuser roller for use in fixing the particulate imaging material to the receiver sheet;
- (c) a supply of offset preventing oil with such offset preventing oil being adapted to react with a zirconia ceramic or its composites to prevent offset of the particulate imaging material;
- (d) a metering roller in contact with the supply of offset preventing oil for wicking such offset preventing oil onto the surface of the metering roller;
- (e) a donor roller in contact with the metering roller and the fuser roller for receiving offset preventing oil from the metering roller and applying it to the surface of the fuser roller; and
- (f) wherein the surface of the metering roller and the surface of the fuser roller are formed from zirconia ceramic or its composites which has a hardness greater than 12 GPa and toughness greater than  $6 \text{ MPa}^{\sqrt{\text{mm}}}$ , and wherein the donor roller is formed from a compliant material.

\* \* \* \* \*